

# United States Patent

[11] 3,616,168

[72] Inventor Paul L. Johnstone  
Greenville, Del.  
[21] Appl. No. 862,130  
[22] Filed Aug. 13, 1969  
[23] Division of Ser. No. 619,739, Mar. 1,  
1967, Pat. No. 3,484,916  
[45] Patented Oct. 26, 1971  
[73] Assignee Hercules Incorporated  
Wilmington, Del.

[56] References Cited  
UNITED STATES PATENTS  
3,003,304 10/1961 Rasmussen ..... 57/157  
3,499,822 3/1970 Rasmussen ..... 264/210 X  
Primary Examiner—Robert F. Burnett  
Assistant Examiner—Roger L. May  
Attorney—William L. Peverill

[54] NONWOVEN FABRIC FROM PLIES OF PLASTIC  
1 Claim, 2 Drawing Figs.  
[52] U.S. Cl. 161/154, 161/402, 264/171, 264/210  
[51] Int. Cl. D04h 13/00, D04h 5/02, D04h 5/08  
[50] Field of Search 161/153, 154, 402; 28/72.2 R, 72.17; 264/210, 171

**ABSTRACT:** This invention relates to a nonwoven fabric made from a plurality of layers of a uniaxially oriented plastic film which are needled by a group of barbed needles to split the film into filaments, with some of the filaments being broken and the ends thereof worked into the fabric, the present invention being characterized by the use of a composite two-ply film which, after needling, is subjected to heat whereby the free ends of the broken filaments will curl because of the uneven shrink characteristics of the two plies and thus cannot readily be pulled from the fabric.



PATENTED OCT 26 1971

3,616,168



FIG. 1

PAUL L. JOHNSTONE  
INVENTOR.



FIG. 2

## NONWOVEN FABRIC FROM PLIES OF PLASTIC

This application is a division of U.S. application Ser. No. 619,739, filed Mar. 1, 1967, now Pat. No. 3,484,916.

The present invention relates to a nonwoven fabric and a method of making the same, and particularly to a nonwoven fabric and method of the type forming the subject matter of my prior U.S. Pat. application Ser. No. 424,646, filed Jan. 11, 1965 and now Pat. No. 3,428,506.

The nonwoven fabric disclosed and claimed in my prior application Ser. No. 424,646 is formed from a film assembly comprising a plurality of superposed plies of plastic film which is passed through a needling or felting machine in which barbed needles are passed through the film assembly. Each ply of film is stretched or oriented in one direction and is preferably arranged with the axis of orientation thereof at right angles to the axes of orientation of adjacent plies of film. While oriented film has great strength in the direction of the axis of orientation, it is quite weak in the direction transverse to the direction of the axis of orientation. Therefore, when the needles penetrate the film, they tend to split the film a short distance in each direction from the needle hole along lines parallel to the direction of the axis of orientation. Each film ply is thus reduced to a filigreelike structure consisting of parallel filaments aligned in the direction of the axis of orientation and connected together at the unsplit portions of the film between alternate penetrations by the needles. In addition to puncturing the film and splitting it outwardly from the needle hole, the barbs of the needles also break some of the filaments to provide ends that are then pushed into the fabric and become intermeshed with other filaments and ends to provide a nonwoven fabric.

The objects of this invention are to provide a nonwoven fabric of the type forming the subject matter of my above noted prior application Ser. No. 424,646, and having improved strength both laterally and between the film plies, which strength is obtained through means that are economical and adapted for commercial operation.

According to the present invention, a film assembly is first formed by superposing a plurality of plies of plastic film, as described in my prior copending application Ser. No. 424,646, except that one or more of said plies comprises a composite film consisting of discrete but intimately adhered layers of two plastic materials having different shrink characteristics. The film assembly is then needled, as described in my prior application, and either simultaneously therewith or subsequent thereto is heated at a temperature that will effect substantial shrinkage of one component of said composite ply or plies and minimal shrinkage of the other component of said ply or plies whereby the filaments of said composite ply will undergo crimping. This tends to lock them more firmly with the filaments with which they are intermeshed and results in a substantial increase in tensile strength of the nonwoven fabric.

Having in mind the above, as well as other objects that will be evident from an understanding of the invention, a preferred embodiment of the present invention is hereinafter disclosed with reference to the accompanying drawings, in which:

FIG. 1 is a schematic view illustrating an apparatus for performing the process and for making the product of this invention.

FIG. 2 is a fragmentary view in section of one of the plies of plastic film that is to be used in accordance with this invention.

With reference to the drawings, there is illustrated in FIG. 1 an apparatus for performing the process and for producing a nonwoven fabric in accordance with this invention. While the number of plies of film may, of course, vary, there are in the illustrated embodiment of the invention 5 plies of identical film identified at 1, 2, 3, 4, and 5, which are supplied from rolls 6, 7, 8, 9, and 10 respectively. The individual plies of film are collected by a pair of opposed feed rollers 11, one of which is driven, into a superposed relation to provide what is herein termed the film assembly 12.

From the feed rollers 11, the film 12 passes between the bed plate 13 and the stripper plate 14 of a needling or felting

machine that also includes a needle bar 15 carrying a plurality of barbed needles 16 that, in the usual manner, may be arranged in rows along the length of the needle bar 15. The needle bar 15 is adapted to be reciprocated by conventional means (not shown) to project the needles 16 through the film assembly 12 and through aligned holes in the stripper plate 14 and bed plate 13. At the output side of the needling machine, there is provided a pair of puller feed rollers 17 which act to advance through the machine the film assembly 12 and the nonwoven or needled fabric 18 produced therefrom.

In the illustrated embodiment of the invention, the needled fabric 18 is subjected to a heat treatment which may be effected, for example, in an oven 19. To advance fabric 18 through the oven 19 there is provided a pair of opposed puller feed rollers 20, one of which is driven. The rollers 20 preferably impose a tension on the fabric 18 between them and the rollers 17, not only to support the fabric 18 by tension within the oven 19, but also to control the endwise shrinkage of the fabric.

The films 1, 2, 3, 4, and 5 are each uniaxially oriented and therefore, because of the inherent weakness of such film in the direction transverse to the axis of orientation, splits in both directions from the needle hole along the axis of orientation as the needle penetrates the film. After successive penetrations by the needles and advancement of the film assembly 12 between each penetration, each film is reduced to a filigreelike structure consisting of a plurality of filaments extending parallel to the axis of orientation and connected to the adjacent filament at the unsplit portions between successive needle penetrations. The length of the splits that are developed by the needle hole can be varied by varying the tension imposed upon the film between the feed rollers 11 and 17.

As the films are split by the needles into a filamentary structure, the filaments are caught to a random fashion by the barbs of the needle and broken to produce ends that are pushed through the adjacent plies of film. In this manner, the ends are thoroughly intermeshed with the filaments and ends of the other plies of the film to form a stable nonwoven fabric. While, for convenience, the above described apparatus includes only a single needle bar 15 that is disposed above the film assembly 12, it will be apparent that a second needle bar disposed beneath the film assembly 12 and operating upwardly therethrough may also be used.

The direction in which the axis of orientation of the various plies of film in the film assembly 12 are arranged may be varied to produce different effects in the fabric, that is, particularly to increase or to decrease the tensile strength of the fabric in any one direction by aligning the axis of orientation of more or less of the films in the selected direction. In a preferred arrangement the axis of orientation of each ply is disposed substantially at right angles to the axes of orientation of adjacent plies.

In accordance with this invention, the film assembly that is used includes one or more plies of a composite film having intimately adhered discrete layers of two different plastic materials, as illustrated at 21 and 22 in FIG. 2. While the specific composite film or the method of manufacturing the same forms no part of this invention, such film may be formed, for example, by bringing the two materials or components together in a molten condition at the die of a film extruder in such a manner that they will be layered and not mixed and simultaneously extruded in a single sheet, which sheet is then expanded and uniaxially oriented in the usual manner. For purposes of this invention, it is required only that the two materials or components of the composite film have significantly different shrink properties at some heat treating temperature. An example of a suitable film is an integrally formed uniaxially stretched film having discrete layers of polypropylene of different molecular weight distribution but of similar melt flow, which is heat treated in the oven 19 at a temperature of about 140° C. At such a temperature, except insofar as it might be restrained for example, between the rol-

lers 17 and 20, one layer shrinks substantially more than the other. Accordingly, there is an uneven shrinkage between the two layers of the filament and the same will therefore be crimped as it is heated in the oven 19.

The manner in which the heat is applied to the fabric can also be varied. While the heat treatment in the illustrated embodiment of the invention is effected in the oven 19, it may also be effected at the time the fabric is needled, as for example, by applying the heat to the fabric through heating the bed plate 13 and stripper plate 14.

The amount of heat that is applied to the fabric is controlled to produce different effects. From the standpoint of improved strength, the individual ends, as well as the filaments themselves, if permitted to assume a crimp, become more firmly interlocked with the ends and filaments with which they are intermeshed. Crimping of the filaments also effects a shrinkage of the fabric which can, to a certain extent, be controlled by placing the fabric under tension as by a longitudinal tension imposed by the rollers 17 and 20 and by a transverse tension imposed by a tenter mechanism (not shown). Accordingly, it will generally be desirable to effect only a limited amount of crimping, or else to tension the fabric to control shrinkage during heating. By exposing only the surface of the fabric to heat, only the filament ends that protrude from or lie on the surface become crimped, which in effect knots these ends and increases their resistance to being pulled back through the fabric. By tensioning the fabric to control shrinkage and by exposing the fabric to heat sufficient to penetrate the same, a thorough crimping of all of the untensioned ends and filaments is effected. By exposing the untensioned fabric to a thorough heating, complete crimping as well as significant shrinkage results.

The materials from which composite films are formed are selected on the basis of their compatibility in the film forming

operation, as well as the difference in their shrinking characteristics. In the film forming operation, if the above-mentioned extrusion process is employed, the polymers must be capable of being simultaneously extruded into a single composite sheet 5 of two distinct integrally formed layers of materials having different shrink characteristics, and subsequently uniaxially oriented. In the crimping operation, the shrink temperatures of the two polymers must be sufficiently different that the differential shrinkage may be performed on a commercial basis. 10 The materials used may, for example, be two polypropylene polymers of different molecular weights and/or molecular weight distributions. More generally, the materials may be polyolefins such as polyethylene, polypropylene, and poly(butene-1); the polyesters such as poly(ethylene terephthalate) 15 and poly(1,4-cyclohexylenedimethylene terephthalate); the polyamides such as nylon sixth-sixths, nylon six-tenths and nylon 6; polystyrene, copolymers of vinylidene chloride and vinyl chloride; poly(vinylidene chloride); poly(vinyl chloride), the polyethers such as poly(ethylene oxide) and 20 poly(propylene oxide), and the like.

What I claim and desire to protect by Letters Patent is:

1. A stable nonwoven fabric composed of a plurality of plies each of which comprises a filigree-like structure consisting of parallel plastic filaments connected to each other at random 25 intervals along the length thereof, some of said filaments in each ply being broken to form ends which protrude through adjacent plies and intermesh with the filaments and ends of said adjacent plies, the filaments of each ply being aligned in a direction different from the alignment of filaments in adjacent 30 plies, and at least one of said plies being composed of adhered layers of two different plastic materials having different shrink characteristics and being crimped as a result of having been heated to cause said layers to shrink to a different degree.